

# UNITED STATES PATENT OFFICE.

JAMES WALLACE PATON, OF SOUTHPORT, ENGLAND.

## MANUFACTURE OF PLATED OR COATED IRON OR STEEL SHEETS.

No. 904,444.

Specification of Letters Patent.

Patented Nov. 17, 1908.

Application filed August 1, 1908. Serial No. 446,464.

To all whom it may concern:

Be it known that I, JAMES WALLACE PATON, subject of the King of Great Britain, residing at Southport, in the county of Lancaster, in the Kingdom of England, have invented certain new and useful Improvements in or Relating to the Manufacture of Plated or Coated Iron and Steel Sheets, for which application has been made in Great Britain, 10 No. 22,028, dated October 5, 1907.

This invention has for its object to produce sheets which will resemble very closely sheets of aluminium or other metal which will take a high polish, and which can be 15 used for almost any purpose for which tinned sheets are used, while at the same time my product is actually cheaper than ordinary tinplate.

In carrying the invention into effect, I 20 take sheets or plates of iron or steel which have first been treated, to confer on them smoothness and elasticity. They are also treated or prepared so as to remove grease, and produce a clean surface to which aluminium varnish will adhere. Any oxidation on 25 the rim or edge of the plate, or on the surface is removed by a sand papering or emery papering machine or equivalent mechanism. These plates I coat on one or both sides with 30 a suitable varnish, preferably in a varnishing machine. I then stove the plates until they become about as tacky as a jujube on a damp day, and apply powdered aluminium all over the surface by means of a dusting 35 machine. While still tacky, the sheet is passed between brushing rollers which distribute the powder evenly over the entire surface, and force it into the varnish evenly. The plates are now left to dry or are a little 40 further stoved, and are then passed through a burnishing machine, where they receive a good polish and finish. This burnishing machine is preferably provided with velvet coated rollers, but I may under some circum- 45 stances pass the sheets first between two smooth steel rollers revolving at different velocities, and then afterwards pass them slowly through the rapidly revolving velvet covered rollers. The plates are finally 50 stoved and are then ready for market. While speaking only of aluminium heretofore, bronze powders, gold, platinum and other powdered metals will produce substantially similar results, and I therefore do not 55 bind myself to aluminium; but aluminium

powder is the cheapest and best for nearly all purposes of this nature. Further, I have simply spoken of varnish; but this varnish can be either transparent and colorless varnish or it can be colored with any desirable 60 coloring matter, and thus delicate tints can be given to the finished article. Plates thus produced I find can be bent, pressed out, stamped, drawn or spun, and punished very 65 greatly without cracking the aluminium layer or removing it from the surface that comes in contact with the dies. Furthermore the plate not having been overheated and brought in contact with hot metal, retains all its original toughness and flexibility. 70

Another advantage the invention has, is that while with tinplate from the very mode in which it is produced, it has to be tinned on both sides, there is no necessity for my plates to be coated on more than one unless 75 required, and thus the cost of coating the plate on the other face is avoided, as it is only the outside of plates used for making many classes of boxes or canisters which are required to be coated. Another advantage 80 of my aluminium coated plates is, that they do not give the peculiar metal taste or smell in handling which is apt to be given by tin.

Hitherto there has been nothing offered as a substitute for tin plate which could be 85 utilized in the same manner as tin plate i. e. which could be drawn or stamped with dies, or printed on to produce the same effect, as a tin plate. If a plate be merely coated with an aluminium paint, made up of aluminium and varnish and allowed to dry, the coating will crack and come off when the plate is bent or stamped, but by my invention, the fact of first varnishing a plate, and then partially stoving and forcing the 90 aluminium into the varnish, and stoving again, and polishing, a coating is produced which for all practical purposes, adheres to the surface as effectually as tin does, and protects the surface from rust, also enables 95 the plate to be used as a substitute for tin plate and at a much less cost. I am also aware that it is already known to apply to the surface of metal a mixture of alumina soap, volatile oils and aluminium or alu- 100 minium bronze powder, and the surface so treated then exposed to the open air or to heat or burned in, or the alumina soap compound was melted upon the metal before the 105 application of the aluminium, and the coat- 110

ing polished. This process is very different from my invention as hereinbefore set forth.

I declare that what I claim is:—

The process of obtaining a brilliant metallic looking surface, which consists in taking a black plate, removing oxidation therefrom especially on the rim or edge, coating it with varnish, allowing the varnish to arrive at the tacky condition, applying the powdered metal, and distributing the powder evenly over the entire surface, at the same time

forcing it into the varnish, afterwards burnishing it in the manner described, and stoving.

In witness whereof, I have hereunto signed 15 my name this 24 day of July 1908, in the presence of two subscribing witnesses.

JAMES WALLACE PATON.

Witnesses:

HUGH WATSON,  
THOMAS S. SHILLINGTON.